

# UNITED STATES PATENT OFFICE.

WALTER RÜBEL, OF CHARLOTTENBURG, GERMANY.

## IRON ALLOY.

1,128,726.

Specification of Letters Patent. Patented Feb. 16, 1915.

No Drawing.

Application filed October 22, 1913. Serial No. 796,671.

*To all whom it may concern:*

Be it known that I, WALTER RÜBEL, a citizen of the Empire of Germany, residing at Reichsstrasse 103, Charlottenburg-West-5 end, in the Empire of Germany, have invented a new and useful Iron Alloy, of which the following is a specification.

The present invention has for its object a novel dynamo iron and a process for manufacturing same. The novel iron is mainly intended for the production of dynamo plates and it is advantageously differentiated from similar known plates owing to the fact that in addition to its excellent 15 electrical properties, it presents favorable mechanical properties such as have never hitherto been obtained.

It is already known to manufacture a relatively efficient dynamo plate by mixing 20 pure iron or iron containing a comparatively small proportion of impurities with a certain percentage of aluminium. By this means eddy or Foucault current losses are almost entirely eliminated. In order to attain this result, the aluminium must be distributed as uniformly as possible between the iron molecules and thinly coat them. As from 1 to 2% of aluminium is sufficient for this purpose, the electrical conductivity 25 is not so much reduced as to render it difficult to magnetize the iron by the current. Consequently, no more ampere windings than with ordinary iron are required. The conditions are different as regards hysteresis 30 however. As is known this phenomenon is explained by the assumption that in the penetration of the electric current and the reversal of the poles in the iron, the molecules are selected in correspondence with 35 the velocity of the reversal of polarization.

This gives rise to frictional heat, the amount of which exactly corresponds with the loss of power experienced in the power employed from the exterior, of course after deducting 40 the small loss due to eddy currents. Accordingly, the greater the freedom of movement of the iron molecules, the smaller is the loss due to hysteresis. This theory is supported by the fact that the loss by 45 hysteresis is smaller when upon reversal of the polarization, the iron body is subjected to quick external hammering. In this case, the decrease of the loss by hysteresis corresponds to the work expended in hammering 50 the iron. The reversal of the iron molecules is even facilitated by the shocks. Con-

sequently, a diminution of the loss by hysteresis could be obtained if the reversal of the iron molecules could be facilitated. This is the case with the iron which forms 60 the object of the present invention owing to the fact that the form of the iron crystals is converted from that of coarse cubes as hitherto into a finely granular form by means of suitable additions which combine 65 with the aluminium and not with the iron. Now it has been found that this result can only be attained and that the best kinds of iron are only produced when silicon is added in addition to the aluminium. The 70 total quantity of aluminium and silicon should not exceed 3% of the iron and the quantity of aluminium should be located between 1 and 2% and the quantity of silicon between 0.8 and 1.2%. This results in 75 an iron alloy which is greatly superior to the known silicon iron plates as regards flexibility, mildness and other mechanical properties. Its magnetizability is very good and quite equal to that of the aluminium 80 iron.

It is known to reduce the loss of wattage by making an addition of silicon to iron. This iron is however, so hard and bristle that it is only with difficulty that it can be 85 rolled out into thin plates so that the cost of manufacturing silicon iron plates is disproportionately high. The mechanical after treatment of these plates also presents difficulties and the wear of the tools employed 90 is very great. The novel iron containing silicon and aluminium in the proportions indicated can readily be rolled and consequently its cost is approximately one half that of the silicon iron plates hitherto 95 known.

Iron containing 1.5% of aluminium and 1% of silicon presents a wattage loss which does not exceed 1.7%. Of this loss 0.15% is due to eddy currents and 1.55% to hysteresis. With 25 ampere windings the magnetizability amounts to 14500. The bending coefficient is however 70 as compared with 6 which is the coefficient of the known silicon plates containing approximately 2% of 100 silicon. The silicon can be replaced by equal quantities of boron with the same satisfactory results. In this case also an extremely fine division of the iron molecules takes place.

In manufacturing the novel kind of iron an iron presenting the maximum degree of 110

purity is produced in any convenient manner such for example as by the combination of an acid and a basic process and the silicon is added to this iron in the form 5 of ferro silicon while the necessary aluminum is added after the deoxidation. It is, however, highly advantageous to introduce the appropriate quantity of aluminum beneath the acid slag upon the bath. In this 10 case, the aluminum reduces silicon from the slag and this silicon passes into the final product combined with the aluminum in excess. Corresponding quantities of beryllium or calcium might be employed in place 15 of the aluminum. These substances are

added to the iron in the form of metal or in the form of an iron alloy.

I claim:

An iron alloy suitable for the manufacture of electric-dynamical machines, containing less than 3% aluminum and silicon, and consisting of iron of 99.5% purity, and of a mixture containing 1-2% aluminum, and 0.8-1.2% silicon, substantially as described. 20

WALTER RÜBEL.

Witnesses:

WOLDEMAR HAUPT,  
HENRY HASPER.